

Dec. 10, 1929.

F. W. MOORE

1,739,322

PILE FACED MATERIAL AND PROCESS OF MAKING THE SAME

Filed Jan. 2, 1924

Fig. 1.



Fig. 4.



Fig. 2.



Fig. 3.



Fig. 6.



Fig. 5.



Fig. 7.



INVENTOR.

Frederick W. Moore,

BY

Arthur G. Jenkins

ATTORNEY.

REISSUED

## UNITED STATES PATENT OFFICE

FREDERICK W. MOORE, OF EAST ORANGE, NEW JERSEY

## PILE-FACED MATERIAL AND PROCESS OF MAKING THE SAME

Application filed January 2, 1924. Serial No. 683,935.

My invention relates to that class of materials used for coverings in upholstery, footwear, apparel and the like, and an object of my invention, among others, is the production of a finish on material of this sort and a process for making it, which material shall possess peculiar characteristics and which process shall enable the material to be produced in a particularly efficient and economical manner.

Material embodying my invention and a process for effecting the purpose of the invention, and in the making and use of which the objects herein set out, as well as others, may be attained, are illustrated in the accompanying drawings in which—

Figure 1 is a perspective view of a portion of a machine illustrating the method of making my improved material.

Figure 2 is a view, scale enlarged, in section through a piece of material illustrating the method of its construction.

Figure 3 is an edge view of a piece of material.

Figure 4 is a diagrammatic view illustrating the manner of producing material with a smooth face.

Figure 5 is a perspective view of a piece of material illustrating the manner of producing a smooth faced material in accordance with my invention, and having a maximum length of pile.

Figure 6 is a view showing a piece of fabric as produced by the patterned roll of Figure 1.

Figure 7 is a view showing the leather applied to the back face of the fabric side of a piece of plush.

Leather, as is well known, is a particularly durable material for use as a covering in upholstery and the like, but it is objectionable on account of its hard and cold feeling. It is believed that if these objectionable features could be removed, leather would be employed to a much greater extent, not only in upholstery, but in various other lines, as in wearing apparel and in other articles requiring durability in wear.

The material illustrated and described herein and embodying my invention com-

prises a leather structure having the desirable features of soft feeling and of warmth desired. The invention also contemplates material other than leather to which a pile facing may be applied as a finish in the manner 55 set out.

In the practice of my invention I take a piece of leather or other material 5 to one side of which I apply a coating of flexible adhesive binder 6, and to which I combine the 60 pile side of a piece of plush 7 or other fabric faced with free erect fleece or fiber in forms to have their ends inserted into the adhesive binder to stand erect therein. In doing this the ends of the fibers 8 comprising the plush 65 face or nap or pile are so set into the adhesive binder as to cause such face to be firmly secured and the structure thus formed is caused to pass between feed rolls 9 and 10, one of which rolls, as 9, may, if desired, have a patterned surface 11. This patterned surface 70 may, however, be omitted when it is desired to produce a material having a smooth face, as shown on roll 16 in Figure 4. The material is moved forward between said rolls 75 to the action of a rapidly moving knife 12 of band construction, which construction will be readily understood by those skilled in the art, and the rolls may be feed rolls or pin rolls.

It is of prime importance that the material shall be moved to the action of the knife with as little compression as possible, but sufficient to maintain it against the cutting action of the knife to feed uniformly at 85 all points and this is accomplished by frictional grip upon the backing in either way produced, that is, whether with a smooth or a patterned face. Therefore, in order to provide for a uniform feed of the material to the knife the rolls, one or both, may be roughened, a pattern on one roll, when such roll is used, providing the necessary roughness for that roll. This frictional grip of the feed rolls upon the material may further be 90 improved by providing a rest roll 13 of soft rubber for one of the feed rolls to impart a frictional pinch pressure to said feed rolls, and an auxiliary pull may be obtained by the action of pin rolls 14 and of fabric rolls 15 95 100

upon the latter of which the material may be wound as it is being divided, the action of said rolls being to pull the material toward the cutting knife. An even thickness of 5 backing substance on both sides of the pile is important to uniform cutting with smooth faced rolls.

While I have hereinbefore described leather as the material having a coating of flexible adhesive binder, the invention contemplates material other than leather, as cloth, 10 felt or other material that may be substituted for the leather, and the backing materials may be arranged in various ways, and they 15 may be applied by means of the adhesive to either or both sides of the plush structure, as for instance, leather may be applied as hereinbefore described to the face of the plush, and the latter being cut as hereinbefore set 20 forth, another piece of leather may be applied by the adhesive to the free ends of the pile, and the latter being then again cut two pieces of leather each with a plush face will be produced, or the leather may be applied 25 to the back surface of the fabric side 17 of the plush structure as shown in Figure 7 of the drawings.

In securing the ends of the plush fibers to the backing of leather or other material, I 30 employ a flexible adhesive binder that is sufficiently plastic to permit the material to be embossed, if desired, this binder having such characteristics as to permit the embossing and at the same time permanently retain the 35 material in its embossed condition. This binder lies between the leather or other material and the pile or fleece, the roots of which are embedded in the adhesive so that the combined material, after it has been cut forms a 40 finish, that may be completed by embossing, and which embossing will be absolutely permanent, and having the leather life, the plush pile, fleece or other face is like a suede and superior in finish to embossed plush, or fabrics which are without the leather body substance. 45

The plastic flexible body which I employ as a binder is composed of cotton nitrates with alcohol or other solvent and combined 50 with vegetable oil, and I have found that the pile of the plush or other material, when anchored in said combining body will produce a material that may be embossed, and the finish will be more permanent than such 55 embossing without the presence of said combining body.

The material is to quite an extent strengthened by the cut pile after it is cut, and being inlaid in its surface fiber this construction and 60 the embossing increases this strength by intermingling portions of the cut fiber with the surface fiber of the leather and the binder combining said fiber to a union therewith and giving material strength to thin or split 65 leather as well as a desirable finish.

While I have illustrated and described herein a plush fabric forming one side only of the structure to be cut I contemplate that the plush fabric, when a patterned surface is to be produced, may comprise both sides of the structure previous to and during the cutting operation. When a roll with a patterned surface, as shown in Figure 1, is employed a fabric having a patterned surface 18 will be produced, as shown in Figure 6, whereas when a smooth roll, as 16, is used, as shown in Figure 4, a fabric with a smooth surface as shown in Figure 5 will be the result, the pile being cut in a direction and so held as to cause the cut to skim along at or near the ends of the fibers and close to that surface of the strip that is to form the face thereof thereby embodying a suede or fur-like face to the same. 70 75 80 85

The fibers comprising the plush face of a piece of plush fabric are all inclined in a certain direction with respect to the backing or woven part of the fabric, and I have found that this feature may be taken into account in the splitting operation, as hereinbefore set 90 forth. From extended experiments I have found that if the material comprising the two backings with the plush fibers between them be moved toward the knife so that the latter will operate against or in a direction opposite to the direction of slant of the fibers projecting from the piece which it is desired shall have the longest fibers composing the face, a distinct advantage will be gained. This is shown in Figure 2 of the drawings in which 95 it will be seen that the knife 12 is operating against or in a direction opposite to the direction of slant of the fibers projecting from the cloth backing 7 which it is desired shall have the longest fibers, the leather backing 5 containing the shorter fibers, and in operating against the fibers as above described, I mean that the fibers shall be inclined toward the knife, as shown in Figures 2 and 4 of the drawings. 100 105 110

In other words, the knife is presented to the fibers in close proximity to either backing the material being cut being presented to the knife so that the shorter fibers will slant away from the knife, as shown in Figures 2 and 5 of the drawings. This enables the knife to be presented to the fibers close to the adhesive on the leather or other backing, in fact, such knife in many instances being presented much closer to the adhesive than shown in Figure 2. A result of this is that the knife after striking the fibers creeps up or rather, the fibers are pressed down so that the knife actually cuts the fibers at a point farther away from the bottom backing than at the point at which the knife first makes contact with the fibers. The knife thus imparts a shearing cut to the fibers and the ends thereof are cut on a slant. The ends thus cut close to or near the face of the fabric or leather 115 120 125 130

compose a uniform dense face upon the fabric having all of the ornate characteristics of fine velvet or suede and the body substance composing the combining medium giving

5 the "feel" and utility of leather.

While I have illustrated herein the cutting as actually taking place between the inner surfaces of the two backing members, it will be understood that my invention contemplates

10 this cutting of the fibers at any point between the outer surfaces of the backing members, even to the extent of cutting through the woven fabric to which the pile is secured or looped, and as shown in Figure 5 of the drawings in which the cutting is shown as being

15 through the loops of the pile.

I claim—

1. That process that consists in arranging the pile filling between more rigid backings

20 in a manner to slant said pile to place one backing forward of the other and at the same time cut through the pile filling between said backings.

2. That process that consists in securing

25 the free ends of the fibers comprising the soft face of a piece of material having a more rigid flexible backing to another backing composed of leather in a manner to cause said fibers to stand erect without distortion,

30 then placing one backing in advance of the other to slant the fibers without material compression and at the same time cutting through the soft material between such backings.

3. That process that consists in securing

35 the free ends of obliquely disposed fibers comprising the soft face of a piece of material with a more rigid flexible backing to another backing also of more rigid flexible material, then placing one of the backings in advance

40 of the other to slant the fibers without material compression and at the same time cutting through said fibers closer to one than the other of said backings and in the direction of slant of said fibers from that backing close

45 to which they are cut.

4. A new article of manufacture comprising a backing of flexible material having a surface of plush inlaid in a flexible cement binder in such manner as to cause the fibers

50 to stand erect and without distortion, said fibers having obliquely cut free ends and the flexible cement binder located between the plush and the backing to secure the inner ends of the fibers comprising the plush pile to the

55 surface of the flexible backing.

5. A new article of manufacture comprising a backing of leather having a coating of cement binder, and a plush pile having the ends of its fibers embedded in said binder

60 and the oppositely obliquely cut ends disposed close to said backing and in the direction of slant of said fibers from said backing to impart a soft face to the leather.

6. A new article of manufacture comprising a backing of flexible material having a

surface of plush fibers inlaid in a flexible cement binder and disposed obliquely and cut short in such a manner as to cause the fibers to stand erect and without distortion, said cut free ends being developed by the cutting to a density to cover the backing, said flexible cement binder being located between the plush and the backing to secure the inner ends of the fibers comprising the plush pile to the surface of the flexible backing and the cement 70

75 imparting the cement consistency to the pile surface.

FREDERICK W. MOORE.

80

85

90

95

100

105

110

115

120

125

130